

## UNITED STATES PATENT OFFICE

2,287,082

## PROCESS FOR THE PRODUCTION OF IRON POWDERS

Karl Bauer, Frankfort-on-the-Main, Germany,  
assignor, by mesne assignments, to Chemical  
Marketing Company Inc., New York, N. Y.

No Drawing. Application November 19, 1938, Serial No. 241,462. In Germany December 16, 1937

3 Claims. (Cl. 204—10)

My invention relates to a process for the production of iron powders.

According to this invention iron powder, which is characterised by its high degree of purity and great reactivity, is prepared by electrolysing a ferrous chloride solution, which contains ammonium salts, for example ammonium chloride, ammonium acetate, or ammonium propionate, in the presence of such quantities of organic acids that the solution has a pH value of 6.5 to 7.2. Formic acid, acetic acid, lactic acid, propionic acid and the like may be employed as organic acids. For many purposes formic acid has proved to be particularly advantageous.

The electrolysis is with advantage carried out with high cathodic current densities, for example current densities of 4 to 10 amperes per dcm.<sup>2</sup>, preferably 6 to 7 amperes per dcm.<sup>2</sup>, advantageously at elevated temperature for example about 50–70° C.

Plates of wrought iron or ingot iron are with advantage used as anode. In the production of the purest iron powder a starting material of corresponding purity is employed, for example one which is free from sulphur and silicon and particularly also of impurities which deposit on the cathode, such as manganese.

Iron plates may likewise be employed as cathode.

The electrolysis is with advantage carried out by causing the electrolytes to flow through a series of cells. When carrying out the electrolysis care must be taken to ensure that the pH value remains within the limits to be maintained according to the invention. The electrolyte has a tendency to become alkaline owing to the action of the current. The properties of the cathode product, for example with regard to texture and solubility, may be thereby changed to an undesired degree.

The cathodically deposited iron, which, after being scraped off from the electrode, is preferably thoroughly washed, and with advantage dried in vacuo at low temperatures, is practically free from carbon and other disturbing impurities. The resulting products depending on the degree of purity of the initial materials, contain for example about 98% and more of metallic iron. Owing to its great hardness the cathode product can be comminuted to any desired degree of fineness, for example in ball mills or edge mills. It is extraordinarily reactive, which is evidenced inter alia by the fact that the iron powder rapidly dissolves at ordinary tempera-

ture in dilute acids, for example hydrochloric acid.

It has been further found that by suitably selecting the acid to be added to the electrolytic solution the reactivity of the iron powder can be considerably influenced. By adding formic acid, for example, an iron powder may be obtained, which can be handled both moist and also dry in the presence of air, but which, when caused to glow at one point by ignition, continues to smoulder in the air. By adding acetic acid, for example, an iron powder may be obtained, which on contact with air can be caused to ignite spontaneously. If desired different organic acids may be added to the electrolytic bath and thereby combined effects may be obtained.

The following examples serve to illustrate how the process of this invention may be carried into effect:

20 1. Such a quantity of formic acid (83–85%) is added to a solution containing 35 gms. of ferrous chloride and 100 gms. of ammonium chloride per litre, that the solution has a pH value of 6.5 to 7.2. About 2–3 gms. of formic acid per litre of electrolyte are required for this purpose. A wrought iron plate free from disturbing impurities is employed as anode and an iron plate is likewise employed as cathode. The solution is electrolysed at 60° C. with a current density of 6–7 amperes per dcm.<sup>2</sup> and a voltage of about 1 to 3. During electrolysis the pH value of the electrolyte is if necessary maintained within the region of 6.5 to 7.2 by further addition of acid. As soon as the cathodic deposit is of the desired thickness the electrolysis is stopped and the deposit removed, thoroughly washed and dried in vacuo at about 60° C. The resulting product can be easily and completely comminuted to degree of fineness such as can be passed through a screen of approximately 130 mesh per cm. in comminuting apparatus, such as edge mills, without the use of protective gas. The powdery product can be handled both moist and also dry in the presence of air. If it is caused to glow at one point by ignition it continues to smoulder in the air.

25 2. Such a quantity of acetic acid is added to a solution containing 30 gms. of ferrous chloride and 120 gms. of ammonium chloride per litre that the solution has a pH value of 6.5 to 7.2. A wrought iron plate free from disturbing impurities is employed as anode and an iron plate is likewise employed as cathode. The solution is electrolysed at 65° C. with a current density of 5–6 amperes per dcm.<sup>2</sup> and a voltage of about 2. During electrolysis the pH value of the elec-

trolyte is maintained within the region of 6 to 7 by the further addition of acid. After 12 hours electrolysis the deposited iron is thoroughly washed in water, dried under the exclusion of air and ground. The material ignites in a moist condition in air.

What I claim is:

1. A process for the production of iron powder of great reactivity, which comprises electrolyzing a ferrous chloride solution containing ammonium chloride at a current density of 6-7 amperes per  $\text{dm}^2$  in the presence of formic acid in such a quantity that the pH value of the solution lies between 6.5 and 7.2.

5 2. A process for the production of iron powder of great reactivity, which comprises electrolyzing a ferrous chloride solution containing a substance selected from the group consisting of ammonium chloride, ammonium acetate and ammonium propionate at a current density of 4-10 amperes per  $\text{dm}^2$  in the presence of a substance selected from the group consisting of formic acid, acetic acid, lactic acid and propionic acid in such a quantity that the pH value of the solution lies between 6.5 and 7.2.

10 3. A process as claimed in claim 2 which is carried out at a temperature of about  $65^\circ\text{C}$ .

KARL BAUER.